

T. G. SELLECK.  
METHOD OF CARBONIZING METAL ARTICLES.  
APPLICATION FILED JAN. 20, 1919.

1,402,449.

Patented Jan. 3, 1922.

2 SHEETS—SHEET 1.



Witnesses:  
William S. Morris

Inventor:  
Theodore G. Selleck  
By Adams Jackson  
Attorneys

T. G. SELLECK.  
METHOD OF CARBONIZING METAL ARTICLES.  
APPLICATION FILED JAN. 20, 1919.

1,402,449.

Patented Jan. 3, 1922.

2 SHEETS—SHEET 2.



Witness:  
William S. Morris

Inventor:  
Theodore G. Selleck  
by Adams & Jackson  
Attorneys.

# UNITED STATES PATENT OFFICE.

THEODORE G. SELLECK, OF MOLINE, ILLINOIS, ASSIGNOR TO DEERE & COMPANY, OF MOLINE, ILLINOIS, A CORPORATION OF ILLINOIS.

## METHOD OF CARBONIZING METAL ARTICLES.

1,402,449.

Specification of Letters Patent.

Patented Jan. 3, 1922.

Application filed January 20, 1919. Serial No. 272,164.

To all whom it may concern:

Be it known that I, THEODORE G. SELLECK, a citizen of the United States, and a resident of Moline, in the county of Rock Island and State of Illinois, have invented a certain new and Improved Method of Carbonizing Metal Articles, of which the following is a specification, reference being had to the accompanying drawings.

10 My invention has to do with the carbonization of soft or low carbon steel for use in the manufacture of soft center steel plow shares or other articles in which it is desirable that the steel have a hard outer surface with a relatively soft backing or center. In the manufacture of plow shares, landsides or moldboards, for example, it is necessary that the surfaces exposed to the soil be quite hard so that they will take a 15 polish, will scour and will not wear rapidly from contact with the earth. These hard outer surfaces are, of course, brittle and will break easily if not reinforced, and, therefore, it is desirable that the hard steel be reinforced and strengthened by a backing or a center layer of tough low carbon steel, and the primary object of my invention is to provide an improved process by which steel suitable for use in the manufacture of plow 20 parts or other articles may be produced. A further object is to provide a process of carbonizing metal articles which will also have the effect of straightening them to remove waves or kinks. In describing my invention I shall do so in connection with the treatment of plow shares, but I wish it to be understood that my improved process may 25 be applied in the treatment of a great variety of other articles, and the reference to plow shares is not intended in any sense as a limitation of the scope of the invention hereinafter claimed.

Heretofore in the carbonization of steel shares to provide them with a soft center 30 the shares are cut from a plate or sheet of soft steel, that is to say, a plate that has a relatively low carbon content. The parts are then placed in containers and packed with a material that is high in carbon, after 35 which the containers are introduced into a furnace where they and their contents are subjected to a high temperature for a sufficient length of time to enable the carbon to penetrate and combine with the steel adjacent to its outer surfaces. The depth to

which the carbon penetrates the metal is governed to some extent by the length of time the steel and the carbon material are subjected to the carbonizing temperature. This process is open to a number of serious 60 objections. In the first place the articles to be treated being packed in containers and introduced cold into the furnace, a considerable time is required for the heat to penetrate to the center of the containers and 65 bring the plates or other articles to the requisite high temperature. This not only lengthens the time required for the treatment, but also increases the expense very materially. Again, the articles nearer the 70 outer walls of the containers and the carbonaceous material surrounding them become hot before those nearer the center of the containers, and, therefore, the process begins to operate first on the articles nearer 75 the walls of the containers. The result is that the latter articles absorb more carbon than those near the center of the containers and are carbonized to a greater depth, thus preventing the production of a uniform 80 product. The use of containers is also objectionable because of the added expense for containers and for the labor of preparing them for introduction into the furnace. These and other objections which might be 85 mentioned are avoided by my invention as will be manifest from the following description thereof.

My improved process generally stated 90 consists in heating the articles to be carbonized to a relatively high temperature before subjecting them to the action of the carbonizing material, thereby insuring a uniformity of condition during the subsequent treatment. After this preliminary 95 heating, which is best done in the same heating chamber where the carbonizing is effected, and during which the articles are not packed in containers and have their surfaces to be carbonized freely exposed to the 100 heat of the furnace, carbonaceous material is introduced and filled in around the articles so that the surfaces of all the articles are equally exposed to the carbonizing gases. A heating chamber separate from the combustion chamber is used so that during the succeeding step of the process the contents of the heating chamber are heated by radiant heat and are not exposed to the 105 products of combustion in the combustion 110

chamber. The carbonizing gases liberated by the heat are, therefore, confined in the heating chamber, so that more accurate regulation, and greater economy and efficiency are realized. The mass is then subjected for the requisite period of time to a carbonizing temperature with the result that the articles are evenly and uniformly carbonized, and the whole process is accomplished in a shorter time than is the case with the best earlier practice. The temperature at which the carbonization is effected is usually from 1400° to 1600° F., and the preliminary heating is preferably from 1000° to 1300° F., but these temperatures may be varied to a considerable extent. As in practicing my improved process no containers are employed, the cost of the containers is saved; the heating period is shortened because there are no containers to absorb heat and interfere with the heating of the articles and the carbonaceous material; greater economy and efficiency are obtained because the carbonizing gases are not wasted but are retained and utilized and as the articles are all of a uniform temperature when subjected to the action of the carbonaceous material the result is a uniform product. While these advantages are realized even with such articles as flat plates or sheets of steel they are realized to a more marked extent in the treatment of small metal objects or irregular pieces such as gears, sleeves, bearings, tools, &c., which are apt to be injuriously affected by unequal heating.

In the practice of my improved process in connection with plates used for shares, moldboards, &c., the plates are introduced into the heating chamber of a suitable furnace so that they stand on edge and are spaced apart a sufficient distance to permit the carbonaceous material to be filled in between and around them and this results in the realization of a further advantage since such plates are usually more or less waved or kinky and when they are stood on edge and spaced apart and then heated to a high temperature they will straighten. This not only improves the condition of the plates themselves, but also permits the carbonaceous material to be introduced evenly and uniformly between them so that the gases generated in the carbonizing step of the operation circulate evenly and have uniform contact with the faces of the plates and substantially the same amount of carbon will be absorbed by the plates throughout their entire face areas.

The preliminary heating not only raises the articles to be treated to a uniform temperature as described, but possesses the further advantage that it expands the metal and opens its pores, so that when the carbonaceous material is introduced and carbon gases are liberated they are not wasted,

but are immediately absorbed by the metal. The gases liberated from the carbonaceous material are produced at a lower temperature than is required to expand the metal and open its pores, and consequently where the carbonaceous material and articles are introduced into the furnace at the same time and while they are relatively cold the gases liberated before the metal reaches the temperature necessary to effect its carbonization will be to a considerable extent lost, whereas by preliminary heating the articles and then introducing the carbonaceous material, as soon as the gases are liberated the metal will be in a condition to absorb them, so that there will be no appreciable waste, and the carbonizing will be more quickly effected. Thus time is saved and economy of carbonaceous material is effected as compared with the old container method in which the carbonaceous material first becomes hot and begins to yield carbon gases before the metal is prepared to absorb the carbon, and, therefore, a surplus of carbonaceous material is required in order that there may be carbonaceous material actively generating gas at the time the metal becomes hot enough to absorb the carbon from the gas. Furthermore, by preliminary heating the articles in the heating chamber in which the subsequent step of carbonization is to be performed, they do not have to be handled while hot, and they are kept hot and in proper condition for the continuation of the treatment.

In the accompanying drawings I have illustrated one form of apparatus which may be advantageously employed in practicing my improved method, which apparatus will form the subject-matter of a separate application for patent, but it will be understood that my improved process may be practiced by the use of other forms of apparatus, as any suitable instrumentalities for practicing it may be employed.

In the accompanying drawings,—

Fig. 1 is a longitudinal vertical section of a furnace showing a charge of plates inserted in the heating chamber, the plates resting upon a truck designed especially for charging the heating chamber and which is withdrawn from under the plates before the doors are closed, leaving the plates in the heating chamber standing on edge and spaced a distance apart;

Fig. 2 is a view similar to Fig. 1 showing the situation after the charging truck has been removed and the heating chamber has been partly filled with the carbonaceous material. This figure also shows thermocouples in place for determining the temperature within the heating chamber;

Fig. 3 is a partial cross-section of the furnace, the truck and plates being shown in elevation; and

Fig. 4 is a view similar to Fig. 3 showing the position of the plates after the truck has been removed.

The furnace is constructed principally of refractory material, such as fire brick, or cement adapted to resist the effect of high temperatures, and it is provided with one or more heating chambers 5 so arranged that the hot gases of combustion do not enter said chambers but are arranged to travel around them except at the ends. The furnace has a foundation 10, side walls 11, end walls 12 and a slightly arched top 13. Extending upwardly from the foundation 10 are transverse piers 14 upon which the heating chambers 5 are supported, and the spaces between the piers constitute flues 15 which are in communication with the main combustion chamber 6 of the furnace. The fuel preferably employed for combustion is oil of a petroleum character. As has been suggested, the furnace may comprise one or more heating chambers 5, and when a series of heating chambers are provided they are separated from each other, and the furnace is so arranged as to cause the gases of combustion to flow around the heating chambers.

Each heating chamber 5 comprises a base 16, side walls 17, a top 18 and a rear wall 19. The front of each heating chamber or compartment is provided with upper and lower doors 7-8 hinged upon the front wall of the furnace, as shown in Figs. 1 and 2. Between the interior side walls of the furnace and the exterior side walls of the adjacent heating chambers at the point most remote from the combustion chamber of the furnace vertical flues 20 are provided to form a passageway for the gases of combustion, as shown in Figs. 3 and 4, these vertical flues being virtually a continuation of the flues 15. After the gases pass through the flues 20 they travel through the space 21 between the top of the heating chambers and the top of the furnace and thence downwardly along the sides of the heating chambers through vertical flues 22 formed between the opposing walls of adjacent heating chambers and vertical partitions 23 which extend down from the roof of the furnace to bases 24 provided between adjacent heating chambers. Where a single heating chamber is provided one of the side walls of the furnace would take the place of the partition 23. The bases 24 are placed directly above the piers 14 and are spaced apart from each other so that the openings between said bases form flues to permit hot gases to pass under the partitions 23 from one vertical flue 22 to the adjacent one, so that the gases continue to travel around the heating chambers until they pass into an evacuating stack 9 located at the combustion chamber side of the last heating chamber of the series. This

construction is best shown in Figs. 3 and 4. Where only one heating chamber is provided the flues formed between the bases 24 are arranged to deliver the gases directly into the evacuating stack.

As best shown in Figs. 1 and 2, the upper doors 7 are arranged to swing about horizontal pivots and the lower doors 8 are arranged to swing about vertical pivots. The upper doors 7 are each provided with a counterbalance lever 26 suitably mounted upon the furnace and arranged to hold said doors open for charging purposes.

27 indicates a series of plates such as are used in the manufacture of plow shares, mold boards, &c. As illustrated in Fig. 1 these plates are introduced into the heating chambers on trucks 28 designed to be run into the heating chambers bearing a load of plates disposed on edge and spaced a distance apart. Preferably the trucks are provided with transverse rollers 28<sup>a</sup> on which the edges of the plates rest so that after the truck has been moved into the heating chamber by holding the plates 27 against endwise movement and pulling on the truck the latter may be withdrawn from under the plates leaving them resting upon the bottom of the heating chamber, as illustrated in Fig. 4. The upper edges of the plates while on the truck and also after the truck has been removed are held spaced apart until the carbonaceous material has been introduced, as hereinafter described, by spreaders 29 provided with fingers which project down between adjacent plates. When a charge of plates has been introduced and the truck withdrawn the heating chambers are closed and sealed, thermocouples 35 being introduced at the ends of the heating chambers for indicating the temperature therein. For this purpose the doors 8 are provided with openings 30 and the rear walls of the furnace and heating chambers are provided with openings 31 adapted to receive the thermocouples which are arranged to project into the heating chamber so that they contact directly with the ends of one or more of the plates therein, thus giving an accurate indication of the temperatures obtained.

32 indicates swinging doors which are arranged to close inclined chutes or passageways 34 provided in the rear walls of the furnace and heating chambers, as shown in Figs. 1 and 2, these passages being provided for the introduction into the heating chambers of carbonaceous material 33, as illustrated in Fig. 2.

Assuming that the heating chamber or chambers have been charged with the plates or other articles to be treated and that they have been closed and sealed, the hot gases resulting from combustion in the furnace pass through the flues and spaces surround-

70

75

80

85

90

95

100

105

110

115

120

130

ing the heating chambers thereby heating said plates. This heating is continued until the plates are uniformly heated to a temperature of approximately 1200° F. which not only opens the pores of the metal for the absorption thereby of the carbon from the carbonaceous gases subsequently liberated in the heating chambers as hereafter described, but also causes the flattening of any waves or kinks in the plates. After the plates have been heated to the desired temperature the rear doors 32 are opened and a mass of carbonaceous material is introduced through the chutes 34 into the heating chambers. As the carbonaceous material enters the heating chambers an attendant working with implements such as rakes, scrapers and hook bars, introduced through the openings of the front doors 7, which have been opened, drags the carbonaceous material forward and works it down in the spaces between the plates. This is continued until the heating chambers are substantially filled and the carbonaceous material has been filled in between and around the plates, the spreaders 29, being then pulled out through the front doors. When a sufficient quantity of carbonaceous material has been introduced to surround and cover the plates the front and rear doors are again closed and sealed and the temperature within the heating chambers is raised to the point of carbonization where it is maintained for a period of time sufficient for the plates to absorb the desired amount of carbon. The front doors 7—8 are then opened, the plates and carbon compound drawn out, and a new charge of plates introduced for a repetition of the process. It will be apparent that the process may be repeated as often as desired without allowing the furnace to cool down or materially reducing the temperature in the heating chambers below that required for the preliminary heating of the plates, so that the work may be carried on very economically.

While in the drawings I have shown the use of a granular carbonizing material it will be understood that my invention is not limited to the use of any particular carbonaceous material, but includes the use of any suitable material, whether powdered, granular or gaseous. Also while I prefer to use fuel oil for heating the furnace any suitable fuel may be employed.

What I claim as my invention and desire to secure by Letters Patent, is—

1. The method of carbonizing metal articles which consists in heating the article to be carbonized by radiant heat before subjecting it to the action of carbonaceous material and afterwards heating the article to a carbonizing temperature in the presence of carbonaceous material.

2. The method of carbonizing metal ar-

ticles which consists in heating the articles by radiant heat in a loose mass in the absence of carbonaceous material and then applying carbonaceous material to and around such articles and subjecting the mass to a carbonizing temperature.

3. The method of carbonizing metal articles which consists in preliminarily heating the article by radiant heat with its surfaces to be carbonized freely exposed to the heat, and afterwards placing carbonaceous material in contact with the surfaces to be carbonized and then heating the article to a carbonizing temperature.

4. The method of carbonizing metal articles which consists in first heating the articles to be carbonized to a high temperature by radiant heat in the absence of carbonaceous material, and then while they are still hot packing carbonaceous material around them and heating the mass to a carbonizing temperature.

5. The method of carbonizing metal articles, which consists in placing the articles loosely in a heating chamber, subjecting the chamber to heat until the articles are uniformly heated to a high temperature, then introducing carbonaceous material into the heating chamber and packing it around the articles, and then heating said chamber by radiant heat to a carbonizing temperature.

6. The method of carbonizing metal articles which consists in introducing the articles into a heating chamber, subjecting the heating chamber to a temperature approximately that of the temperature of carbonization until the articles are uniformly heated, then introducing into the heating chamber and around the articles a carbonaceous material, and then subjecting the heating chamber to a higher temperature for a period of time sufficient to cause the articles to absorb carbon from the carbonaceous material.

7. The method of carbonizing metal articles which consists in introducing the articles to be treated loosely into a suitable heating chamber closed against the admission of the products of combustion so that they are directly exposed to the heat thereof, heating the articles in the absence of carbonaceous material, afterwards introducing carbonaceous material into such chamber into direct contact with such articles, closing said chamber, and then heating the mass to a carbonizing temperature.

8. The method of carbonizing metal articles which consists in introducing the articles to be treated loosely into a suitable heating chamber so that they are directly exposed to the heat thereof, and heating such articles in the absence of carbonizing material, afterwards packing carbonaceous material around the articles, and then heating the mass to a carbonizing temperature.

9. The method of carbonizing metal plates which consists in heating the plates to a relatively high temperature while standing on edge and afterwards heating the 5 plates to a carbonizing temperature in the presence of carbonizing material.
10. The method of carbonizing metal plates which consists in standing the plates on edge in a suitable heating chamber and 10 heating them to a relatively high temperature in the absence of carbonizing material, then introducing a carbonizing material into the heating chamber, and then heating the plates to a carbonizing temperature.
11. The method of carbonizing metal plates which consists in standing the plates on edge spaced apart from each other in a suitable heating chamber, and heating 20 them to a relatively high temperature, then introducing a carbonizing material into the heating chamber, and then heating the plates to a carbonizing temperature.
12. The method of carbonizing metal plates which consists in standing the plates on edge spaced apart in a suitable heating chamber, then heating them to a relatively high temperature by radiant heat, then introducing a carbonizing material into the 25 heating chamber, and then heating the mass to a carbonizing temperature.
13. The method of carbonizing metal
- plates which consists in standing the plates on edge spaced apart in a suitable heating chamber, then heating them to a relatively high temperature in the absence of carbonizing material, then introducing a solid carbonizing material into the heating chamber between and around said plates, and then heating the mass to a carbonizing temperature.
14. The method of carbonizing metal articles which consists in placing the articles to be treated spaced apart in a heating chamber and afterwards introducing 35 into the heating chamber and into direct association with the articles to be treated a suitable solid carbonizing material and subjecting the mass to a carbonizing temperature for a time sufficient to cause the absorption by the articles of carbon from the carbonizing material.
15. The method of carbonizing metal articles which consists in placing the articles to be treated spaced apart in a heating 40 chamber, heating the chamber to a high temperature in the absence of carbonizing material, and afterwards introducing into the heating chamber and into direct association with the articles to be treated a suitable solid carbonizing material and subjecting the mass to a carbonizing temperature.

THEODORE G. SELLECK.